

April 29, 1941.

J. B. HUDSON

2,239,784

REAR PROJECTION SCREEN

Filed April 25, 1938



INVENTOR  
JESSE B. HUDSON

BY

Ward, Crosby & Neal  
ATTORNEYS

## UNITED STATES PATENT OFFICE

2,239,784

## REAR PROJECTION SCREEN

Jesse B. Hudson, Philadelphia, Pa., assignor to  
 Trans-Lux Corporation, New York, N. Y., a corporation of Delaware

Application April 25, 1938, Serial No. 204,139

3 Claims. (Cl. 88—24)

My invention relates to a rear projection screen, i. e., a screen of the type wherein the projecting light beam passes through the screen while passing from the projector mechanism to the auditorium area or the like.

In accordance with my invention, there is produced a screen of the rear projection type which comprises an oiled fabric suitably treated to render the same properly light-diffusive for the intended purpose.

Further objects, advantages and characteristics of my invention will appear from the following detailed description.

My invention resides in the rear projection screen, the method of producing the same together with the features of procedure of the character hereinafter described and claimed.

For an understanding of my invention and for an illustration of one form thereof, reference is to be had to the accompanying drawing, in which the figure is an enlarged, sectional view showing a screen as constructed in accordance with my invention.

In accordance with a preferred form of my invention, there is produced a structure S of sheet-like character having the function of serving as a screen or surface for the display of projected images. The aforesaid screen or surface is disposed, usually, substantially vertically between the auditorium area and the projector mechanism, the beam of light from the projector mechanism passing to the auditorium area after traversing said screen or surface.

A screen or surface constructed in accordance with my invention may be produced in a variety of ways. Thus, as a coating medium for suitable fabric f such, for example, as natural silk, artificial silk or other suitable material, it has been demonstrated that there may be utilized a more or less transparent mixture formed principally from linseed oil, with which is combined other suitable oils and ingredients such as cellulose esters, synthetic resins and plasticisers as desired. After the screen fabric f, in suitable manner, has had applied thereto a coating of the character described and, after such coating had dried to suitable extent, there is applied to the coated fabric surface a medium d utilizable as a light diffuser.

As one example of a substantially transparent

coating medium which yields satisfactory results in accordance with my invention, a satisfactory formula is set forth as follows:

|                                                           | Parts by volume |
|-----------------------------------------------------------|-----------------|
| Linseed oil                                               | 80              |
| Chinawood oil                                             | 4               |
| Fish oil                                                  | 2               |
| Dryer (manganese dioxide, cobalt oxide, lead oxide, etc.) | 3               |
| Plasticiser (tri-cresyl phosphate, tri-phenyl phosphate)  | 1               |
| Resins                                                    | 5               |
| Cellulose esters                                          | 5               |

The linseed oil (boiled) has the other formula ingredients mixed therewith and then, in suitable manner as by dipping a tautly held sheet of fabric f in a bath formed from the coating medium, said coating medium is applied to the fabric after the latter has been sized. Thereafter, in suitable manner, the fabric f is maintained taut usually for many hours so that the coating medium may harden or set and, if necessary, this action may be hastened by placing the tautly held treated fabric in a heated atmosphere.

After the coating medium has set to a desired extent and, while it is still somewhat tacky, the light-diffusive agent d, in accordance with the invention, is applied to the coated fabric surface. To this end, light-diffusive material d such as corn starch, talcum powder, zinc oxide, zinc stearate, titanium oxide, or the like may be evenly distributed, as by sprinkling, an air blast operation, or the like on such coated fabric surface. The amount of the light-diffusive material d which is thus utilized is dependent upon the light-transmission factor which the completed screen is to have although, in general, it will be understood that the quantity of said light-diffusive material d is such that the screen diffuses the light in a proper manner when it is included in a rear projection system.

After the light-diffusive material d has thus been applied all at one time or by successive operations to one or both faces of the coated fabric f, the latter is maintained taut until completely dry whereupon it may be cut to form screen sections of a desired size. The screen sections may be suitably bound at their edges,

as well understood in the art, before they are assembled in their respective frames.

When a fabric is coated as described above, the oxidizing oil, in addition to its desirable refractive function and that of placing the fabric in condition for use as a screen, tends, in an undesired manner, to cause the screen to become hard or stiff as it ages. As a result, if the plasticizer was not incorporated, brittleness and cracks would eventually develop in the screen, the plasticizer, therefore, insuring pliability of the screen despite the above noted tendency of the oxidizing oil.

The use of fish oil as a part of the coating medium is desirable because it serves somewhat as a plasticiser to cause the completed screen to be relatively flexible and pliable.

Under some circumstances, it may be desirable to incorporate other oils or materials in the above described coating medium. Thus, it may be desirable to include in said coating medium a small quantity of Perilla oil which, somewhat the same as the Chinawood oil, causes the coated surface to be tougher and to more readily "take" the subsequently applied light-diffusive material. Further, if desired, a small quantity of soya bean oil may be incorporated in the coating medium, such oil serving to restrain the treated fabric from turning yellow. Also, as generally stated above, it may be desirable to add to the coating medium one or more cellulose ethers such as ethyl cellulose or one or more cellulose esters such as cellulose acetate, etc. and also certain organic synthetic resins.

It is to be distinctly understood that my invention is not to be limited to the formula herein described in detail since it will be understood by those skilled in the art that the proportions of the specified materials may be varied within reasonable limits and, moreover, some of the specified materials may be omitted and others supplied, if desired, to thereby produce a coating medium having desired characteristics.

While the invention has been described with respect to certain particular preferred examples which give satisfactory results, it will be understood by those skilled in the art after understanding the invention, that various changes and modifications may be made without departing from the spirit and scope of the invention and it is intended therefore in the appended claims to cover all such changes and modifications.

What is claimed as new and desired to be secured by Letters Patent is:

1. A rear projection screen comprising a fabric sheet, a coating medium for said fabric sheet, said coating medium being a mixture comprising linseed oil principally together with Chinawood oil and fish oil to considerably less extent, said coating medium, after application to said fabric sheet, causing the surface thereof to be in tacky condition, and powdered light-diffusive material applied externally to the coated surface of said fabric sheet, said light-diffusive material serving to overcome the tacky condition of said fabric sheet, said light-diffusive material and said fabric sheet serving to diffuse the light of the projecting light beam while permitting the passage of sufficient light for rear projection practice.

2. A rear projection screen comprising a fabric sheet, a coating medium for said fabric sheet, said coating medium being a mixture comprising linseed oil principally together with Chinawood oil, fish oil, soya bean oil and Perilla oil to considerably less extent, said coating medium, after application to said fabric sheet, causing the surface thereof to be in tacky condition, and powdered light-diffusive material applied externally to the coated surface of said fabric sheet, said light-diffusive material serving to overcome the tacky condition of said fabric sheet, said light-diffusive material and said fabric sheet serving to diffuse the light of the projecting light beam while permitting the passage of sufficient light for rear projection practice.

3. A rear projection screen comprising a fabric sheet, a coating medium for said fabric sheet, said coating medium being a mixture comprising by volume linseed oil principally together with about three parts of a dryer, substantially less than three parts of a plasticiser, Chinawood oil, a resin and a cellulose ester each approximately in the same proportion and each somewhat greater in volume than that of the dryer, and fish oil in volume somewhat less than that of the dryer, said coating medium, after application to said fabric sheet, causing the surface thereof to be in tacky condition, and light-diffusive material applied exteriorly to the tacky coated surface of said fabric sheet, said light-diffusive material serving to overcome the tacky condition of said fabric sheet, said light-diffusive material and said fabric sheet serving to diffuse the light of the projecting light beam while permitting the passage of sufficient light for rear projection practice.

JESSE B. HUDSON.